

April 23, 1957

P. D. NORA, JR

2,789,895

METHOD OF AGGLOMERATING FINE IRON ORES

Filed May 19, 1954

3 Sheets-Sheet 1



FIG. 1



FIG. 2

INVENTOR.  
PETER D. NORA, JR

BY

*J.R. Harris*  
ATTORNEY

April 23, 1957

P. D. NORA, JR

2,789,895

METHOD OF AGGLOMERATING FINE IRON ORES

Filed May 19, 1954

3 Sheets-Sheet 2



FIG. 3



FIG. 4

INVENTOR.  
PETER D. NORA, JR  
BY

*J.R. Harris*

ATTORNEY

April 23, 1957

P. D. NORA, JR

2,789,895

METHOD OF AGGLOMERATING FINE IRON ORES

Filed May 19, 1954

3 Sheets-Sheet 3



FIG. 5

INVENTOR.  
PETER D. NORA, JR  
BY

*J.R. Harris*

ATTORNEY

2,789,895

**METHOD OF AGGLOMERATING FINE IRON ORES**

**Peter D. Nora, Jr., Negaunee, Mich., assignor to Jones & Laughlin Steel Corporation, Pittsburgh, Pa., a corporation of Pennsylvania**

Application May 19, 1954, Serial No. 430,793

6 Claims. (Cl. 75—5)

This invention relates to the agglomeration of finely divided metalliferous materials and more specifically to the agglomeration of iron ores and iron ore concentrates.

Although my invention is applicable to finely divided metalliferous materials generally, it is particularly adapted to the agglomeration of iron ores and will be described as applied to such materials. Finely divided iron ores, especially those resulting from various concentration or beneficiation processes are not suited to conventional blast furnace reduction, as they tend to form a dense burden in the furnace shaft through which the blast finds its way with difficulty. Various methods have been proposed and tried for processing such finely divided ores, flue dust, and the like into discrete particles or masses of larger size. These include sintering, briquetting, nodulizing, pelletizing, and other agglomerating processes, of which only sintering is widely employed. The sintering process consists of mixing ore properly moistened with a small amount of fuel such as coke breeze, coal fines, and the like, spreading the mixture in a uniform layer over a grate, igniting it, generally at the top, and causing combustion of the fuel to proceed through the bed by drawing air through the charge. The heat developed partially fuses or agglomerates the charge into a sinter cake which breaks up into lumps of substantial size.

The conventional sintering process makes it possible to agglomerate into a satisfactory blast furnace feed ores much finer than those which can be successfully smelted directly in the blast furnace. However, very finely divided ores, such as result from the fine grinding necessary to liberate so-called martite and taconite ores from gangue particles, are not well adapted to agglomeration by conventional sintering. This is because the sintering process requires that air be drawn through the unsintered charge and very fine ores tend to form a closely packed bed having low air permeability.

It is an object, therefore, of my invention to provide a process by which such finely divided iron ores can be sintered. It is another object of my invention to provide a sinter having a novel structure. Further objects will appear in the course of the following description and explanation of my invention.

As I have mentioned, my invention is particularly applicable to finely divided iron ore concentrates. A screen analysis of such an ore concentrate to which my invention is applicable is given in Table I.

Table I.—Screen analysis

| Tyler screen size: | Percent weight retained |
|--------------------|-------------------------|
| 200 mesh           | 4.81                    |
| 325                | 16.35                   |
| 400                | 2.14                    |
| —400               | 76.70                   |

Table I indicates that more than three-quarters of this concentrate was minus 400 mesh size. The principal chemical constituents of this concentrate are set out in Table II.

Table II.—Chemical analysis

|                                | Percent |
|--------------------------------|---------|
| Fe                             | 63.62   |
| FeO                            | 27.25   |
| Fe <sub>2</sub> O <sub>3</sub> | 60.69   |
| SiO <sub>2</sub>               | 5.44    |
| Al <sub>2</sub> O <sub>3</sub> | 3.53    |

It is known to agglomerate ores and ore concentrates such as that described above into more or less spherical particles called pellets. This may be done by introducing the ore and a measured amount of water into a drum rotating about an axis inclined slightly to the horizontal. As the material passes through this drum it balls up or forms more or less spherical pellets, the size of which can be controlled within a considerable range without too much difficulty. Pellets of suitable size, say one inch or more in diameter, can be charged directly into a blast furnace if they can be made strong enough to withstand the weight of the charge in the furnace shaft. The wet pellets coming from the drum are quite plastic and in this condition will support very little weight without deforming or disintegrating. The physical strength of such pellets is considerably increased by drying and may be further increased by heating them to elevated temperatures. Such drying or heating requires apparatus especially constructed for such purpose and is a rather tedious process, however, since rapid heating turns the moisture in the pellets to steam, causing them to disintegrate.

I have found that pellets formed as described above can be sintered in a conventional sintering machine such as a Dwight-Lloyd or a Greenawalt machine, and that the product so formed has a novel structure. I have found that pellet disintegration can be prevented and that moisture-containing pellets can be successfully sintered if the properties of the moist pellets are controlled and the bed of pellets on the grate of the sintering machine is covered with a layer of unagglomerated iron ore in a manner to be described.

It is known to add a certain proportion of ore as pellets, granules or briquettes, to a sinter mix in the same manner as return sinter fines are added with the object of improving the permeability to air of the bed of sinter mix. Usually the ore below some selected screen size is agglomerated and added in this way to the mix of coarser ore particles. A bed of sinter mix so formed may show a higher permeability to air than a bed of similar ore conventionally prepared. This increase in bed permeability disappears, however, as soon as sintering begins. My invention differs markedly from such known practices in that the great bulk of the sintering machine charge is in the form of pellets, and these are not mixed with unagglomerated ore.

The first step in my process is the mixing with the finely divided iron ore of a small proportion of carbonaceous fuel. This fuel may be of any type conventionally used in sintering and should be added in amount less than that sufficient to sinter the ore in the conventional manner. In conventional sintering of iron ores, fuel equal to about 6% to 8% of the charge weight is added to the ore. I have found that fuel in amounts between 2% and 4% of the weight of the ore is sufficient for my pellets, and that this amount, although too low to ignite by itself, will provide enough heat to sustain sintering if sintering is commenced by the ignition of an upper layer of ore richer in fuel. If fuel much beyond 4% is added, the pellets will fuse to such an extent that the passage of air through the charge is hindered. It is desirable that the fuel be ground to a reasonable fineness so that it will mix uniformly with the finely divided iron ore. Minus 65 mesh coal is satisfactory.

The mixture of ore and fuel is then formed into pellets in

a horizontally rotating drum in the manner known to the art. Sufficient water must be introduced into the drum, usually in the form of a spray, to enable the ore to ball satisfactorily. The amount of water necessary ranges from about 10% to about 20% of the weight of the ore. Most ores contain an appreciable amount of water, and those beneficiated by wet processes may contain enough water to form pellets without any further moistening. I prefer to use pellets averaging about one-quarter inch in diameter and not larger than about three-eighths inch, as pellets much larger than this require an extended time for thorough sintering. The pellets should not be so small that they pack firmly on the grate and reduce the bed permeability to air. I find that pellets which are held on a 6 mesh Tyler screen are about the smallest which can be satisfactorily sintered. The openings in such a screen are .131 inch square.

The moisture-containing pellets direct from the pelletizing drum may then be spread directly upon the grate of a conventional sintering machine. As these wet pellets do not have great mechanical strength, the depth of the bed must not be so great that the weight of the upper layers deforms the pellets at the bottom. If this occurs, the pellets at the bottom spread out and form a layer of low air permeability, thus slowing down the sintering operation. For wet pellets about one-quarter inch size of the concentrate of Table II the pellet bed depth should not exceed about 5 inches, to permit the application of an upper layer as described below. It will be understood, however, that a bed of pellets of this depth weighs as much as a considerably deeper bed of coarse ore because of the compacting of the fine ore in the pelletizing operation.

On top of the pellet bed so formed I then form a layer of a conventional sinter mix of iron ore and fuel. The ore may be the same finely divided ore from which the pellets are formed or it may be a coarser ore. Return fines may also be included in this layer, if desired. The fuel content of this layer should be sufficient to ignite but need not be more. I find that fuel amounting to about 8% by weight of the layer is sufficient. The size of the fuel incorporated in this layer is not critical. I find that minus one-quarter inch coke is a satisfactory fuel. The weight of this upper layer should not be less than about 5% of the weight of the pellet bed and may be more, if desired, up to the weight at which bed permeability to air is adversely affected or the bottommost pellets are deformed. I have had good success with upper layers amounting to one-third the weight of the pellet bed when the upper layer was highly permeable to air. In general, however, the great bulk of the charge should be in the form of pellets. The fuel in the upper layer is then ignited and the charge sintered in the conventional manner.

I find that a charge prepared as above described can be sintered considerably more rapidly than the same weight of the same type of ore of a particle size range well adapted for conventional sintering. In one installation with which I am familiar a charge prepared in accordance with my invention as above described was sintered in seventeen minutes, whereas a conventional charge of the same weight required thirty-three minutes for sintering. I believe this increased speed of sintering is attributable to the relatively great permeability to air of the pellet bed of my invention. The wet pellets could not have been sintered at all, however, without the upper layer, which appears to transfer heat to the pellets below in the form of combustion gases in such manner that the pellets dry without spalling or disintegrating.

My process is facilitated if the grates of the sintering machine before being charged with my pellets are first covered with a thin layer of coarse ore, return fines, or dried or semi-hardened pellet fragments. For convenience I designate such material "coarse ore-like particles." The presence of a hearth layer of coarse ore-like particles appreciably increases the permeability to air of the charge.

apparently by permitting excess moisture at the bottom of the charge to drain away from the bottommost pellets. If hot return fines from the sintering operation are used in this hearth layer, the bottommost pellets charged on to it are partially dried and hardened, thus increasing the depth of bed they can support.

A significant advantage of my process is the saving in fuel it makes possible. As I have mentioned, conventional sintering requires fuel equal to about 6% to 8% of the charge weight. My process requires this proportion of fuel for the upper layer only, but the pellets forming the remainder of the charge and accounting for perhaps three-quarters or more of its weight require only 2% to 4% of their weight as fuel.

15 My invention provides sinter of novel structure and properties. These are illustrated in the attached figures to which reference is now made.

Figure 1 illustrates two sections of sinter cake, the sections being the full height of the cake which resulted from 20 the sintering of a 4½ inch pellet bed plus a 1½ inch upper layer.

Figure 2 shows three random pieces of sinter from a broken sinter cake.

Figure 3 is a photomicrograph at a magnification of 25 300 diameter of a section through sinter of my invention.

Figure 4 is a similar photomicrograph at the same magnification of conventional hard sinter.

Figure 5 is a graph illustrating the comparative resistance to crushing of the sinter of my invention and conventional hard and soft sinter.

It will be observed that the sinter illustrated in Figures 1 and 2 is formed of a large number of individual pellets fused sufficiently to join together but not so much that their identities have disappeared.

35 The microstructure of my sinter is shown in Figure 3. In this figure the individual ore grains 1 are clearly visible. Most of these grains 2—2 are in direct contact with one another and are bonded by particle-to-particle fusion. The darker colored constituent 3 visible in many grains is 40 magnetite; the lighter colored constituent 4 is hematite formed by oxidation of magnetite. The gray constituent 5 is slag. The black areas 6—6 are pits or voids in the specimen.

The microstructure of conventional hard magnetite 45 sinter is shown in Figure 4. Here none of the grains 1 is in direct contact with another, but all these grains, which are magnetite, are bonded by the slag matrix 5. The black areas 6, again, are pits.

Figures 3 and 4 demonstrate that my sinter contains substantially less slag than conventional hard sinter and that nearly all the grains in my sinter are directly bonded together without the intervention of any slag. Because of this desirable structure, my sinter is as easily reduced in the blast furnace as the best conventional soft sinter.

55 The terms "hard" and "soft" as applied to sinter refer primarily to its physical strength, particularly its resistance to crushing. Hard sinter is made by extending the time of sintering, or increasing the fuel content of the sinter mix, or both, so that more complete fusion of the mix 60 is obtained and a mechanically strong sinter is produced. Such sinter does not easily crush under the load of the burden in a blast furnace, and a substantial "hardness" of this type is desired by blast furnace operators. It is recognized, however, that sinter "hardness" is conventionally attained, however, at the expense of reducibility. "Soft" sinter is less completely fused than "hard" sinter and is mechanically weaker, but is more easily reduced in the blast furnace.

Figure 5 illustrates graphically the results of crush 70 tests performed on conventional hard sinter, conventional soft sinter, and the sinter of my invention. These tests were performed in the manner described in the paper "Laboratory studies on iron ore sintering and testing," by F. M. Hamilton and H. F. Ameen, published in the Transactions of the American Institute of Mining and Metal-

surgical Engineers, Volume 187, December 1950, Mining Engineering, pages 1275-1282. The sinter to be tested is placed in a hollow shell in which is inserted a plunger or anvil. A weight of 150 pounds is dropped on this anvil from a height of 53½ inches. The material is then removed and screen analyzed. The particle size distribution so attained is plotted on the graph of Figure 5. The graph for the pellet sinter of my invention is seen to fall intermediate those for conventional hard and soft sinter, showing that my sinter, though not as hard as conventional hard sinter, is much harder than soft sinter. As has been mentioned, however, my sinter is as easily reduced in the blast furnace as conventional soft sinter.

I claim:

1. The method of agglomerating finely divided iron ore comprising forming a moist mixture of said ore and finely divided carbonaceous fuel in amount insufficient to sinter said ore, forming said mixture into pellets of an average diameter not exceeding about three-eighths of an inch, spreading said moisture-containing pellets in a bed of a depth less than that depth which causes crushing of the moist bottom pellets, spreading on said pellet bed an upper layer of iron ore mixed with carbonaceous fuel in amount sufficient to ignite and sinter said upper layer,

igniting said upper layer and sintering said pellet bed from the top down.

2. The method of claim 1 in which the weight of the upper layer is not less than about 5% of the weight of the pellet bed.

3. The method of claim 1 in which the fuel content of the pellets is between about 2% to about 4% of their weight.

4. The method of claim 1 in which the pellets are 10 larger than six mesh.

5. The method of claim 1 in which the fuel content of the upper layer does not exceed about 8% of its weight.

6. The method of claim 1 in which the moisture-containing pellets are spread on a hearth layer of coarse ore-like particles.

References Cited in the file of this patent

UNITED STATES PATENTS

|    |           |                |               |
|----|-----------|----------------|---------------|
| 20 | 2,582,386 | Komarek et al. | Jan. 15, 1952 |
|    | 2,608,481 | Royster        | Aug. 26, 1952 |
|    | 2,631,941 | Cole           | Mar. 17, 1953 |
|    | 2,672,412 | Burrow         | Mar. 16, 1954 |